

**3,405,016**  
**HEAT TREATABLE TITANIUM BASE ALLOYS**  
**AND METHOD**

Robert I. Jaffee, Worthington, and Horace R. Ogden, Columbus, Ohio, assignors, by mesne assignments, to Crucible Steel Company of America, Pittsburgh, Pa., a corporation of New Jersey

No Drawing. Continuation-in-part of application Ser. No. 520,357, July 6, 1955. This application Apr. 11, 1956, Ser. No. 577,461

3 Claims. (Cl. 148—133)

This invention pertains to titanium-base alloys of novel composition and proportions, which are heat treatable by quenching for imparting relatively low yield strengths to facilitate forming operations, and which may thereafter be strengthened by cold working and aging or precipitation hardening. The invention also pertains to methods of heat treating such alloys for imparting the properties aforesaid.

This application is a continuation-in-part of our co-pending application Ser. No. 520,357, filed July 6, 1955, now abandoned which is in turn a continuation-in-part of our applications Ser. Nos. 122,576, filed Oct. 20, 1949, now Patent No. 2,726,954; 305,284, filed Aug. 19, 1952, now Patent No. 2,798,806; 392,052, filed Nov. 13, 1953, now abandoned; 393,578, filed Nov. 23, 1953, now Patent No. 2,796,347; 396,756, filed Dec. 7, 1953, now Patent No. 2,797,996; 400,730, filed Dec. 28, 1953, now abandoned; 400,744, filed Dec. 28, 1953, now Patent No. 2,779,677; 409,252, filed Feb. 9, 1954, now abandoned, and 470,510 filed Nov. 22, 1954, now abandoned.

There are many applications in which a large spread between yield strength and ultimate strength is desirable in an alloy. For example, when alloys are to be plastically formed to shapes, as by forging, rolling, extruding, drawing, etc., it is desirable to have a low yield strength so that the forming operation can be accomplished more easily. Also, it is desirable to strengthen the alloy after forming by a simple aging heat treatment.

We have discovered that there is a certain class of titanium-base alloys that can be heat treated to produce low yield strengths before forming. These are alloys

which contain both substitutional alpha stabilizers and beta stabilizers, the beta-stabilizer content being less than the critical amount required to produce mechanically stable beta phase on quenching from the all-beta temperature field. There are certain composition limits which must be met before the desired properties are obtained. Also, it is necessary to use a prescribed heat treatment to have the alloys in the correct condition to display this low-yield-strength, high-ultimate-strength property. The alloys of the present invention when quenched from the all-beta and mixed alpha-beta temperature field produce a yield strength to ultimate tensile strength ratio of between about 0.25 and 0.75.

In most beta-stabilized, titanium-alloy systems, there is a composition range in which the beta phase transforms to martensite when the alloy is quenched from the all-beta temperature field. At alloy contents just above this range, the beta phase can be retained by quenching. This beta phase is, however, unstable, and, in most systems, it is hardened by the formation of a coherent precipitate during the quenching process. It has been found that the addition of an alpha stabilizer, such as aluminum, tin or antimony, to alloys containing this beta-stabilizer content, prevents the formation of the coherent precipitate during the quench. The resultant alloy as quenched from the beta temperature field, has a soft beta structure, a very low yield strength, a high ultimate strength and good bend ductility. The beta structure will transform to martensite on cold working, or it can be age hardened to high strength levels.

The compositional limits of the soft beta phase having the large spread between yield strength and ultimate strength will vary according to the beta-stabilizing elements used. It has already been stated that the alloy must contain a substitutional alpha stabilizer in addition to the beta stabilizer. The alpha-stabilizer content may range from 1 to 10% for aluminum, 1 to 23% for tin, or 1 to 19% for antimony, or combinations thereof, tin being replaceable by antimony, and vice versa on a substantially equal percentage basis, and antimony and tin being substitutable for aluminum in the proportion of about 3% of tin and/or antimony for 1% of aluminum. The beta-stabilizer content for alloys quenched from the

TABLE I.—MECHANICAL PROPERTIES OF BETA-QUENCHED Ti-BASE ALLOYS

| Alloy No. | Composition<br>Percent,<br>Balance Ti | Heat Treatment <sup>1</sup> |               | p.s.i.×1,000                    |                   | Percent<br>Elongation<br>in 1" | Percent<br>Red. in<br>Area | Percent<br>MBR, T<br>(Long.) | VHN |
|-----------|---------------------------------------|-----------------------------|---------------|---------------------------------|-------------------|--------------------------------|----------------------------|------------------------------|-----|
|           |                                       | Time,<br>hr.                | Temp.,<br>°C. | 0.2%<br>Offset<br>Yield<br>Str. | Ult. Str.<br>Str. |                                |                            |                              |     |
| A-478     | 5 Al-4 Mo                             | 1                           | 950           | 133                             | 150               | 2                              | 4                          | Br                           | 383 |
| A-477     | 5 Al-5 Mo                             | 1                           | 950           | 105                             | 143               | 10                             | 7                          | 4.5                          | 363 |
| A-452     | 5 Al-6 Mo                             | 1                           | 950           | 90                              | 140               | 12                             | 20                         | 0.8                          | 332 |
| A-453     | 5 Al-8 Mo                             | 1                           | 950           | .57                             | 143               | 10                             | 15                         | 2.5                          | 303 |
| A-454     | 5 Al-10 Mo                            | 1                           | 950           | 46                              | 136               | 9                              | 11                         | 1.5                          | 265 |
| A-455     | 5 Al-12 Mo                            | 1                           | 950           | 87                              | 132               | 5                              | 7                          | 0.7                          | 288 |
| A-456     | 5 Al-14 Mo                            | 1                           | 950           | 105                             | 110               | 16                             | 30                         | 0                            | 272 |
| A-421     | 5 Al-2.5 Mn                           | 1                           | 975           | 119                             | 136               | 14                             | 21                         | 2.1                          | 325 |
| A-422     | 5 Al-5 Mn                             | 1                           | 975           | 152                             | 165               | 5                              | 5                          | Br                           | 394 |
| A-466     | 5 Al-6.5 Mn                           | 1                           | 975           | 72                              | 76                | 0                              | 0                          | 4.7                          | 338 |
| A-423     | 5 Al-7.5 Mn                           | 1                           | 950           | 48                              | 134               | 7                              | 0                          | 1.4                          | 292 |
| A-467     | 5 Al-8.5 Mn                           | 1                           | 950           | -----                           | 114               | 0                              | 0                          | Br                           | 317 |
| A-424     | 5 Al-10 Mn                            | 1                           | 950           | 97                              | 97                | 0                              | 0                          | Br                           | 325 |
| A-391     | 5 Al-2.5 Cr                           | 1                           | 975           | 125                             | 139               | 3                              | 3                          | 2.7                          | 383 |
| A-392     | 5 Al-5 Cr                             | 1½                          | 925           | 68                              | 146               | 14                             | 21                         | 0.4                          | 294 |
| A-481     | 5 Al-6 Cr                             | 1½                          | 950           | 67                              | 158               | 10                             | 17                         | 5.6                          | 387 |
| A-392     | 5 Al-7.5 Cr                           | 1½                          | 875           | 39                              | 128               | 11                             | 18                         | 0.3                          | 282 |
| A-465     | 5 Al-8.5 Cr                           | 1                           | 925           | 111                             | 122               | 6                              | 14                         | 2.2                          | 342 |
| A-394     | 5 Al-10 Cr                            | 1½                          | 850           | 115                             | 120               | 3                              | 5                          | 0                            | 300 |
| A-395     | 5 Al-12.5 Cr                          | 1½                          | 850           | 118                             | 120               | 3                              | 7                          | 0                            | 309 |
| A-406     | 5 Al-15 Cr                            | 1½                          | 850           | 133                             | 134               | 17                             | 27                         | 0                            | 320 |
| A-445     | 5 Al-2 Fe                             | 1                           | 975           | 120                             | 142               | 10                             | 25                         | 0.7                          | 359 |
| A-446     | 5 Al-3 Fe                             | 1                           | 975           | 153                             | 166               | 5                              | 5                          | Br                           | 480 |
| A-447     | 5 Al-4 Fe                             | 1                           | 975           | 50                              | 127               | 6                              | 6                          | 3.0                          | 349 |
| A-448     | 5 Al-5 Fe                             | 1                           | 950           | 99                              | 108               | 2                              | 4                          | 3.6                          | 359 |
| A-449     | 5 Al-6 Fe                             | 1                           | 950           | -----                           | 104               | 0                              | 3                          | Br                           | 344 |
| PA-626    | 9 Sn-7.5 Mo                           | 1                           | 850           | 43                              | 130               | 10                             | 17                         | 1.7                          | 284 |
| PA-627    | 9 Sn-10 Mo                            | 1                           | 850           | 114                             | 134               | 15                             | 38                         | 0.8                          | 302 |
| PA-1412   | 4 Sb-12 Mo                            | 1/4                         | 760           | 69                              | 110               | 8                              | 26                         | 1.0                          | 251 |
| PA-637    | 9 Sn-5 Cr                             | 1                           | 850           | 52                              | 120               | 15                             | 23                         | 0.8                          | 298 |
| PA-638    | 9 Sn-10 Cr                            | 1                           | 850           | 129                             | 130               | 16                             | 31                         | 0.9                          | 330 |

<sup>1</sup> Quenched from temperature.

beta field may have the following ranges or combinations thereof: 5 to 15% molybdenum, 15 to 20% vanadium, 6 to 8% manganese, 4 to 10% chromuminum, and 4 to 5% iron.

Tensile data on beta-quenched alloys, showing the large spreads between yield strengths and ultimate strengths for alloys within these limits, are given in Table I.

As shown by the above data, the most effective compositions for producing a large spread between yield and ultimate strengths are those containing about 8 to 10% molybdenum, about 7 to 8% manganese, about 7 to 8% chromium and about 4% iron.

It is not necessary to quench these alloys from the beta field to obtain the high spread between yield and ultimate strengths. Quenching from a temperature in the alpha-beta temperature field, so that the beta phase retained at room temperature has a composition within the limits described above, will produce the same effect. Examples of this effect are given in the following Table II, which contains tensile data for alloys quenched from the alpha-beta field:

quenched condition. Obviously, the beta-stabilizer content cannot exceed the maximum specified above for each alloying element; as otherwise the beta-phase composition will exceed that of the desired ranges. The minimum beta-stabilizer content to produce an alpha-beta structure in the quenched condition is the lower effective limit for alpha-beta-quenched alloys, producing alpha-beta alloys on quenching. This minimum limit is 1% for each of molybdenum, manganese, chromium and iron, and 2% for vanadium. Thus, this invention is applicable to alpha-beta alloys having beta-stabilizer contents of 1 to 15% molybdenum, 2 to 20% vanadium, 1 to 8% manganese, 1 to 10% chromium, and 1 to 5% iron in addition to the alpha promoters specified previously.

This heat treatment can be used on commercial heats of titanium alloys provided they have the prescribed compositions. For example, the Ti-4Al-4Mn alloy can be heat treated to have a large spread between yield and ultimate strengths by quenching from about 900° C. When quenched from this temperature, the manganese content of the beta phase is of the appropriate composi-

TABLE II.—MECHANICAL PROPERTIES OF TITANIUM ALLOYS QUENCHED FROM THE ALPHA-BETA FIELD

| Alloy No. | Composition<br>Percent<br>Balance Ti | Heat<br>Treatment <sup>1</sup> |               | p.s.i. $\times 1000$            |              | Percent<br>Elongation<br>in 1" | Percent<br>Red. in<br>Area | MBR, T<br>(Long.) | VHN |
|-----------|--------------------------------------|--------------------------------|---------------|---------------------------------|--------------|--------------------------------|----------------------------|-------------------|-----|
|           |                                      | Time,<br>hr.                   | Temp.,<br>°C. | 0.2%<br>Offset<br>Yield<br>Str. | Ult.<br>Str. |                                |                            |                   |     |
| A-485     | 5 Al-5 Mo                            | 5                              | 800           | 105                             | 146          | 6                              | 10                         | 7.8               | 356 |
| A-485     | 5 Al-5 Mo                            | 2                              | 850           | 95                              | 156          | 8                              | 10                         | 3.9               | 352 |
| A-477     | 5 Al-5 Mo                            | 1                              | 950           | 106                             | 143          | 10                             | 7                          | 4.5               | 363 |
| A-486     | 5 Al-7 Mo                            | 8                              | 775           | 125                             | 133          | 13                             | 21                         | 7.5               | 355 |
| A-486     | 5 Al-7 Mo                            | 3                              | 825           | 68                              | 153          | 12                             | 15                         | 2.8               | 309 |
| A-480     | 5 Al-7 Mo                            | 1                              | 950           | 96                              | 149          | 10                             | 7                          | Br                | 358 |
| A-483     | 5 Al-4 Cr                            | 1                              | 875           | 93                              | 158          | 15                             | 13                         | 1.6               | 393 |
| RS-523-39 | 5 Sn-5 Mo                            | 2                              | 750           | 66                              | 111          | 15                             | 51                         | 0.5               | 268 |
| RS-523-40 | 5 Sn-10 Mo                           | 2                              | 750           | 64                              | 112          | 8                              | 30                         | 0.9               | 255 |
| A-405     | 10 Al-2.5 Fe                         | 3½                             | 975           | 65                              | 113          | 4                              | 4                          | 6.6               | 421 |
| RS-523-69 | 5 Sn-5 V                             | 4                              | 750           | 79                              | 116          | 14                             | 27                         | 0.8               | 254 |
| RS-523-60 | 5 Sn-10 V                            | 4                              | 750           | 68                              | 114          | 17                             | 25                         | 0                 | 294 |
| RS-523-65 | 4 Al-5 V                             | 4                              | 750           | 94                              | 133          | 16                             | 29                         | 1.5               | 272 |
| RS-523-57 | 4 Al-10 V                            | 4                              | 750           | 66                              | 132          | 10                             | 25                         | 1.3               | 259 |
| RS-523-64 | 4 Al-2.5 V-2.5 Mo                    | 4                              | 750           | 130                             | 146          | 8                              | 25                         | 2.1               | 328 |
| RS-523-62 | 5 Sn-5 Mo-5 V                        | 4                              | 750           | 72                              | 109          | 20                             | 38                         | 1.1               | 306 |

<sup>1</sup> Quenched from temperature. <sup>2</sup> Quenched from the beta field.

As shown by the above data, a typical example is the Ti-5Al-5Mo alloy. When this alloy is quenched from 800° C., the molybdenum content of the beta phase is above the optimum 10%. When quenched from 850° C., the molybdenum content of the beta phase is closer to the optimum 10%, and a very low yield strength spread is obtained, the properties being very similar to an alloy of this same analysis, as quenched from the beta field, the results of which latter, copied from Table I, are repeated in Table II for comparison. Another example is the Ti-5Sn-5Mo alloy quenched from 750° C., which has an alpha-beta structure, the beta phase of which contains about 10% molybdenum. The properties of this alloy, as shown in Table II, are very similar to the Ti-5Sn-10Mo alloy quenched from the beta field, which, of course, has a molybdenum content of 10% in the beta phase.

Where the alloys are quenched from the alpha-beta field, it is not necessary to limit the alloy content to the ranges specified previously. For this condition, the requirements are: (1) that the quenching temperature in the alpha-beta field is in all instances selected such that the retained-beta phase has a composition within the limits above specified for the beta stabilizers, respectively, as quenched from the beta field, i.e., within 5 to 15% molybdenum, 15 to 20% vanadium, 6 to 8% manganese, 4 to 10% chromium, and 4 to 5% iron, and (2) that the alloy have a two-phase alpha-beta structure in the

50 tion (about 6 to 7%) so that the stresses required to cause flow are very low. This is shown by the data in the following Table III, where it can be seen that the yield strengths of the various heats tested are much lower in the 900° C. quenched condition than in other conditions.

TABLE III.—TENSILE PROPERTIES OF A TI-4Mn-4Al ALLOY QUENCHED FROM VARIOUS TEMPERATURES IN THE ALPHA-BETA FIELD

| Heat Treatment <sup>1</sup> | Temp., °C. | Time, hr. | 0.2% Offset Yield Strength, p.s.i. | Ultimate Strength, p.s.i. | Percent Elongation in 1" | Percent Red. in Area |
|-----------------------------|------------|-----------|------------------------------------|---------------------------|--------------------------|----------------------|
|                             |            |           |                                    |                           |                          |                      |
| Heat B-5306                 |            |           |                                    |                           |                          |                      |
| 790                         | 2          |           | 149,100                            | 156,100                   | 21                       | 42.5                 |
| 840                         | 2          |           | 150,500                            | 156,900                   | 17                       | 36.8                 |
| 900                         | 2          |           | 90,200                             | 178,400                   | 14                       | 10.2                 |
| 950                         | 2          |           | 111,400                            | 132,100                   | 3                        | 1.7                  |
| Heat BN-44056               |            |           |                                    |                           |                          |                      |
| 840                         | 2          |           | 127,000                            | 147,300                   | 13.2                     | 16.8                 |
| 900                         | 2          |           | 74,200                             | 174,300                   | 6.0                      | 5.0                  |
| 950                         | 2          | (?)       |                                    |                           |                          |                      |
| Heat Treatment <sup>1</sup> |            |           |                                    |                           |                          |                      |
| Temp., °C.                  |            | Time, hr. | Compressive Yield Strength, p.s.i. |                           |                          |                      |
| Heat B-31399                |            |           |                                    |                           |                          |                      |
| 870                         |            | 2         | 143,200                            |                           |                          |                      |
| 885                         |            | 2         | 134,900                            |                           |                          |                      |
| 900                         |            | 2         | 83,700                             |                           |                          |                      |

<sup>1</sup> Quenched from temperature.

<sup>2</sup> Brittle.

Additional test data illustrative of the above are given in the following Table IV for molybdenum containing alloys as betal quenched, i.e., as solution treated one hour at 870° C. and water quenched.

In addition to providing a condition whereby the alloys can be readily formed to shapes because of the low yield strengths and good bend ductility, the aforesaid quenching heat treatment can be used as a solution-

TABLE IV.—EFFECT OF SOLUTION-HEAT TREATMENT ON THE PROPERTIES OF Ti-Sn-Mo Ti-Al-Mo AND Ti-Sn-Al-Mo BETA ALLOYS

| Composition percent (Balance Titanium) | Tensile Properties: p.s.i. $\times 1,000$ |                   |                | Elongation, Percent | Percent Red. in area | MBR, T (Trans.) | VHN |
|----------------------------------------|-------------------------------------------|-------------------|----------------|---------------------|----------------------|-----------------|-----|
|                                        | 0.2% Offset Yield Strength                | Ultimate Strength | Total Strength |                     |                      |                 |     |
| 18 Sn-8 Mo                             | 118                                       | 124               | 11             | 3                   | 36                   | 0.75            | 284 |
| 16 Sn-12 Mo                            | 123                                       | 124               | 11             | 3                   | 36                   | 0               | 285 |
| 16 Sn-8 Mo                             | 112                                       | 118               | 18             | 3                   | 36                   | 0               | 282 |
| 14 Sn-16 Mo                            | 118                                       | 121               | 9              | 3                   | 30                   | 0               | 289 |
| 14 Sn-12 Mo <sup>1</sup>               | 114                                       | 116               | 16             | 2                   | 36                   | 0               | 283 |
| 14 Sn-10 Mo                            | 115                                       | 120               | 17             | —                   | 50                   | 0               | 287 |
| 14 Sn-6 Mo                             | 41                                        | 137               | 11             | 7                   | 15                   | 1.1             | 273 |
| 12 Sn-12 Mo                            | 117                                       | 121               | 18             | 2                   | 45                   | 0               | 290 |
| 12 Sn-10 Mo                            | 89                                        | 124               | 9              | 8                   | 31                   | 1.4             | 270 |
| 12 Sn-8 Mo                             | 61                                        | 134               | 8              | 6                   | 13                   | 0.45            | 259 |
| 10 Sn-12 Mo                            | 117                                       | 122               | 14             | 3                   | 37                   | 0               | 275 |
| 10 Sn-10 Mo                            | 87                                        | 119               | 11             | 10                  | 46                   | 0.5             | 262 |
| 10 Sn-8 Mo                             | 43                                        | 123               | 11             | 8                   | 24                   | 0.9             | 257 |
| 9 Sn-6 Mo                              | 74                                        | 125               | 14             | 13                  | 19                   | —               | 294 |
| 8 Sn-12 Mo                             | 94                                        | 109               | 15             | 14                  | 38                   | 0               | 253 |
| 8 Sn-10 Mo                             | 38                                        | 100               | 20             | 8                   | 49                   | 0.5             | 312 |
| 8 Sn-8 Mo                              | 65                                        | 125               | 11             | 8                   | 13                   | 0.55            | 269 |
| 8 Sn-6 Mo                              | 81                                        | 123               | 15             | 14                  | 23                   | —               | 295 |
| 5 Sn-15 Mo                             | 138                                       | 142               | 6              | 2                   | 34                   | 0               | 320 |
| 4 Sn-12 Mo                             | 66                                        | 99                | 38             | 31                  | 48                   | 0               | 257 |
| 4 Sn-10 Mo                             | 66                                        | 105               | 33             | 30                  | 40                   | 5.0             | 260 |
| 4 Sn-8 Mo                              | 67                                        | 127               | 16             | 16                  | 12                   | 9.0             | 320 |
| 3 Sn-6 Mo                              | 88                                        | 121               | 12             | 12                  | 15                   | 0               | 305 |
| 12 Mo                                  | 97                                        | 112               | 10             | 10                  | 12                   | 10              | 330 |
| 10 Mo                                  | 106                                       | 121               | 22             | 22                  | 20                   | 6.6             | 325 |
| 8 Mo                                   | 72                                        | 126               | 17             | 17                  | 28                   | 2.2             | 300 |
| 4 Al-16 Mo                             | 125                                       | 129               | 12             | 3                   | 36                   | 0               | 299 |
| 3 Al-12 Mo                             | 76                                        | 124               | 7              | 6                   | 5                    | 1.2             | 289 |
| 2 Al-8 Mo                              | 72                                        | 118               | 18             | 10                  | 32                   | 3.4             | 280 |
| 4 Al-4 Sn-16 Mo                        | 130                                       | 137               | 11             | 3                   | 32                   | 0               | 315 |
| 3 Al-10 Sn-12 Mo                       | 125                                       | 133               | 13             | 1                   | 35                   | 1.5             | 312 |
| 3 Al-8 Sn-12 Mo                        | 125                                       | 130               | 12             | 1                   | 35                   | 0               | 292 |
| 3 Al-4 Sn-12 Mo                        | 114                                       | 131               | 11             | 4                   | 27                   | 1.2             | 300 |
| 2 Al-8 Sn-8 Mo                         | 46                                        | 145               | 10             | 7                   | 17                   | 1.4             | 278 |
| 2.67 Al-8 Sn-8 Mo-8 Cu                 | 116                                       | 134               | 13             | 10                  | 21                   | 9.2             | 337 |
| 2.67 Al-8 Sn-4 Mo-6 Cu                 | 74                                        | 132               | 6              | 6                   | 20                   | 2.0             | 296 |
| 2.67 Al-8 Sn-4 Mo-4 Cu                 | 79                                        | 147               | 14             | 10                  | 9                    | 1.5             | 323 |
| 2 Al-8 Sn-8 Mo-6 Cu                    | 122                                       | 125               | 6              | 2                   | 14                   | 0               | 295 |
| 2 Al-8 Sn-8 Mo-4 Cu                    | 111                                       | 114               | 7              | 3                   | 32                   | 0.9             | 301 |
| 2 Al-8 Sn-8 Mo-2 Cu                    | 91                                        | 133               | 10             | 7                   | 28                   | 1.9             | 308 |
| 2.67 Al-8 Sn-4 Mo-6 Mn                 | 68                                        | 150               | 15             | 11                  | 24                   | 3.0             | 293 |
| 2.67 Al-8 Sn-3 Mo-3 Mn                 | 71                                        | 143               | 10             | 8                   | 6                    | 1.4             | 289 |
| 2 Al-8 Sn-8 Mo-6 Mn                    | 121                                       | 123               | 18             | 3                   | 36                   | 0               | 297 |
| 2 Al-8 Sn-8 Mo-3 Mn                    | 87                                        | 168               | 11             | 10                  | 4                    | 1.6             | 298 |
| 2 Al-8 Sn-8 Mo-2 Fe                    | 125                                       | 125               | 12             | 3                   | 36                   | 0               | 313 |
| 2 Al-8 Sn-8 Mo-6 Cr                    | 121                                       | 121               | 19             | 3                   | 34                   | 0               | 309 |
| 2.67 Al-8 Sn-4 Mo-8 FeCr               | 135                                       | 137               | 7              | 3                   | 18                   | 1.2             | 333 |
| 2.67 Al-8 Sn-4 Mo-4 FeCr               | 113                                       | 116               | 5              | 3                   | 8                    | 4.8             | 319 |

<sup>1</sup> Average of tests from three melts.

As will be seen from the above data in Table IV, these molybdenum containing alloys may be divided into two groups, namely, those which show little or no tendency to strain transformation as beta quenched, and those showing an appreciable tendency toward strain transformation as beta quenched. The former are characterized by high yield strength and low uniform elongation, and the latter by low yield strength or high uniform elongation or both. Those of both groups are amenable to good formability in the solution-heat-treated condition.

annealing treatment prior to aging. The beta phase in this heat-treated condition is subject to precipitation hardening when heated at temperatures in the range of 300 to 550° C. Thus, an alloy within the prescribed compositional limits can be heat treated to have a low yield strength and good bend ductility by quenching from the appropriate temperature. After quenching, the alloy can be formed into shape and then aged to the desired strength level. Examples of the properties in the quenched condition and in aged conditions of some representative alloys are given in the following Table V.

TABLE V.—PROPERTIES OF QUENCHING AND AGED Ti-BASE ALLOYS

| Composition, Percent (Balance Titanium) | Quenching Treatment |            | Aging Treatment |            | p.s.i. $\times 1000$   |           | Percent Elongation in 1" | Percent Red. in Area | MBR, T (Long.) |
|-----------------------------------------|---------------------|------------|-----------------|------------|------------------------|-----------|--------------------------|----------------------|----------------|
|                                         | Time, hr.           | Temp., °C. | Time, hr.       | Temp., °C. | 0.2% Offset Yield Str. | Ult. Str. |                          |                      |                |
| 4 Al-10 V (RS-523-57)                   | 4                   | 750        | 4               | 500        | 66                     | 132       | 10                       | 25                   | 1.3            |
|                                         | 4                   | 750        |                 | 500        | 167                    | 181       | 3                        | 14                   | 3.2            |
|                                         | 4                   | 750        |                 | 500        | 180                    | 186       | 3                        | 13                   | 3.0            |
| 5 Sn-5 Mo-5 V (RS-523-62)               | 4                   | 750        | 4               | 500        | 72                     | 109       | 20                       | 38                   | 1.1            |
|                                         | 4                   | 750        |                 | 500        | 179                    | 194       | 2                        | 4                    | 8.2            |
|                                         | 4                   | 750        |                 | 500        | 154                    | 171       | 8                        | 15                   | 4.8            |
| 5 Sn-10 Mo (RS-523-39)                  | 2                   | 750        | 4               | 500        | 64                     | 112       | 8                        | 30                   | 0.9            |
|                                         | 2                   | 750        |                 | 500        | 176                    | 189       | 2                        | 9                    | 5.0            |
|                                         | 2                   | 750        |                 | 500        | 176                    | 176       | 5                        | 19                   | 2.8            |
| 5 Sn-5 V (RS-523-69)                    | 4                   | 750        | 4               | 500        | 79                     | 116       | 14                       | 27                   | 0.8            |
|                                         | 4                   | 750        |                 | 500        | 121                    | 136       | 6                        | 19                   | 1.8            |
|                                         | 4                   | 750        |                 | 500        | 111                    | 127       | 9                        | 20                   | 1.7            |
| 4 Al-5 V (RS-523-55)                    | 4                   | 750        | 4               | 500        | 94                     | 133       | 16                       | 29                   | 1.5            |
|                                         | 4                   | 750        |                 | 500        | 127                    | 146       | 14                       | 27                   | 2.7            |
|                                         | 4                   | 750        |                 | 500        | 133                    | 156       | 11                       | 11                   | 2.0            |
| 4 Al-2.5 V-2.5 Mo (RS-523-64)           | 4                   | 750        | 4               | 500        | 130                    | 146       | 8                        | 25                   | 2.1            |
|                                         | 4                   | 750        |                 | 500        | 138                    | 154       | 7                        | 23                   | 3.6            |
|                                         | 4                   | 750        |                 | 500        | 147                    | 160       | 5                        | 15                   | 2.5            |
| 3 Sn-6 Mo (RS-1439-48)                  | 1                   | 870        | 16              | 550        | 88                     | 121       | 12                       | 15                   | -----          |
|                                         | 1                   | 870        |                 | 550        | 169                    | 175       | 1                        | 3                    | -----          |
| 6 Sn-6 Mo (RS-1439-49)                  | 1                   | 870        | 16              | 550        | 81                     | 183       | 15                       | 23                   | -----          |
|                                         | 1                   | 870        |                 | 550        | 172                    | 176       | 2                        | 15                   | -----          |
| 9 Sn-6 Mo (RS-1439-50)                  | 1                   | 870        | 16              | 550        | 74                     | 125       | 14                       | 19                   | -----          |
|                                         | 1                   | 870        |                 | 550        | 167                    | 167       | 1                        | 6                    | -----          |
| 8 Sn-10 Mo (RS-1439-33)                 | 1                   | 870        | 16              | 540        | 38                     | 100       | 20                       | 49                   | -----          |
|                                         | 1                   | 870        |                 | 540        | 149                    | 165       | 4                        | 16                   | -----          |
| 10 Sn-10 Mo (RS-1439-34)                | 1                   | 870        | 16              | 510        | 87                     | 119       | 11                       | 46                   | -----          |
|                                         | 1                   | 870        |                 | 510        | 157                    | 172       | 5                        | 14                   | -----          |
| 12 Sn-10 Mo (RS-1439-35)                | 1                   | 870        | 16              | 540        | 89                     | 124       | 9                        | 31                   | -----          |
|                                         | 1                   | 870        |                 | 540        | 141                    | 158       | 6                        | 24                   | -----          |
| 14 Sn-10 Mo (RS-1439-30)                | 1                   | 870        | 16              | 510        | 115                    | 120       | 17                       | 50                   | -----          |
|                                         | 1                   | 870        |                 | 510        | 181                    | 190       | 3                        | 14                   | -----          |
| 4 Sn-12 Mo (RS-1439-36)                 | 1                   | 870        | 16              | 510        | 66                     | 99        | 38                       | 48                   | -----          |
|                                         | 1                   | 870        |                 | 510        | 168                    | 170       | 2                        | 5                    | -----          |
| 8 Sn-12 Mo (RS-1439-37)                 | 1                   | 870        | 16              | 540        | 94                     | 109       | 15                       | 38                   | -----          |
|                                         | 1                   | 870        |                 | 540        | 137                    | 150       | 4                        | 19                   | -----          |
| 10 Sn-12 Mo (RS-1439-29)                | 1                   | 870        | 16              | 540        | 117                    | 122       | 14                       | 37                   | -----          |
|                                         | 1                   | 870        |                 | 540        | 144                    | 155       | 7                        | 16                   | -----          |
| 12 Sn-12 Mo (RS-1439-28)                | 1                   | 870        | 16              | 510        | 117                    | 121       | 18                       | 45                   | -----          |
|                                         | 1                   | 870        |                 | 510        | 173                    | 179       | 4                        | 16                   | -----          |
| 12 Sn-12 Mo (RS-1439-26)                | 1                   | 870        | 16              | 540        | 117                    | 121       | 3                        | 9                    | -----          |
|                                         | 1                   | 870        |                 | 540        | 194                    | 203       | 2                        | 6                    | -----          |
|                                         | 1                   | 870        |                 | 480        | 114                    | 118       | 17                       | 45                   | -----          |
| 5 Sn-15 Mo (RS-1439-43)                 | 1                   | 870        | 16              | 510        | 138                    | 142       | 6                        | 34                   | -----          |
|                                         | 1                   | 870        |                 | 510        | 180                    | 180       | 1                        | 4                    | -----          |
|                                         | 1                   | 870        |                 | 480        | 211                    | 216       | 1                        | 5                    | -----          |
| 3 Al-10 Sn-12 Mo (RS-1439-31)           | 1                   | 870        | 16              | 510        | 125                    | 133       | 13                       | 35                   | -----          |
|                                         | 1                   | 870        |                 | 510        | 204                    | 206       | 3                        | 9                    | -----          |
|                                         | 1                   | 870        |                 | 480        | 196                    | 200       | 2                        | 10                   | -----          |
|                                         | 1                   | 870        |                 | 480        | 161                    | 166       | 7                        | 20                   | -----          |

Another ingot analyzing 5.4% aluminum, 3.4% vanadium, balance titanium of commercial purity, as water quenched from 820° C., has a 0.2% offset yield strength of 118,000 p.s.i., an ultimate strength of 142,000 p.s.i., an elongation of 16% and an area reduction of 50.5%. On subsequent aging at 890° F. for eight hours, the corresponding values were: yield strength 144,000 p.s.i., ultimate strength 163,000 p.s.i., elongation 9% and area reduction 23%.

The alloys of the invention are further characterized by a rapid increase in work-hardening rate during cold working. This rapid work hardening occurs after an initial period of low work hardening. It is believed to be the results of martensite formation of alpha from beta, which is accompanied by increased hardness and strength. Thus, the alloys can be highly work hardened or strengthened. This is a further mechanism whereby the strength of the alloys may be increased, augmenting the aging mechanism described previously.

Summarizing the above data, it is seen that certain titanium-base alloys can be heat treated to have very low yield strengths. In this heat-treated condition, the 60 alloys can be fabricated or formed to shape and subsequently age-or precipitation-hardened to high strength levels. The requirements for such alloys are: (1) the alloy must contain an alpha stabilizer, such as aluminum, tin and antimony, and also a beta stabilizer. The beta-65 stabilizer content cannot exceed 15% for molybdenum, 8% for manganese, 10% for chromium, 5% for iron, or 20% for vanadium, or proportionate combinations of the above. It is preferable that the beta-stabilizer content be less than the optimum to produce the largest 70 spread between yield and ultimate strengths when quenched from the beta field. This is 10% for molybdenum, 7.5% for manganese, 7.5% for chromium, 4% for iron, or 15% for vanadium. When these alloys contain less than the optimum amount of beta-stabilizing 75 elements, they must be quenched from a temperature

in the alpha-beta field at which the beta phase of the alloys alloys is of the optimum composition; (2) the heat treatment given the alloys is a quench from the temperature at which the beta phase is a composition within the limits described above; and (3) subsequent to quenching, the alloys may be fabricated to shape and then aged to high strength levels by reheating to 300 to 550° C. for periods of time from a few minutes to several days.

All of the alloys, test results for which are given in Tables I to V, inclusive, were produced by arc melting the alloying constituents in a cold mold furnace in an inert or argon atmosphere. The alloys thus produced were thereafter forged in air at about 980° C. and thereupon hot rolled into sheet of about 40 mil gauge at about 700 to 925° C.

Also in Tables I to V, inclusive, the alloys designated "A" were produced from high purity or "iodide" base titanium, obtained by the process set forth in the Van Arkel Patent No. 1,671,213; while those designated "PA" or "RS" were produced from titanium of commercial purity as obtained by the magnesium reduction of titanium tetrachloride in accordance with the patent to Kroll No. 2,205,854.

The beta transus temperature varies with the alloying constituents and content of each, and can be determined for any particular analysis by quenching specimens from the progressively higher temperatures and observing the microstructure. When the betal transus temperature is obtained, the specimen will quench to an all-beta microstructure, whereas on quenching from lower temperatures, some alpha phase will be present.

What is claimed is:

1. A method for producing a titanium-base alloy article having a relatively low yield strength and a relatively high ratio of ultimate tensile strength to yield strength, comprising heat-treating a titanium-base alloy consisting of at least one alpha stabilizer selected from the group consisting of 1 to 10% aluminum, 1 to 23% tin, 1 to 19% antimony, and at least one beta stabilizer selected from the group consisting of 1 to 15% molybdenum, 2 to 20% vanadium, 1 to 8% manganese, 1 to 10% chromium and 1 to 5% iron to a temperature about that at which said alloy shows a minimum point on its yield strength, solu-

tion heat treating temperature curve, and rapidly quenching to produce a yield strength to ultimate tensile strength ratio of between 0.25 and 0.75.

5 2. A titanium-base alloy article produced in accordance with the method of claim 1.

3. A method for solution heat treating a thin section product composed of an alloy consisting essentially of aluminum in amount from about 1 to about 8%, a beta stabilizer selected from the group consisting of chromium in amount from about 2 to about 10%, iron in amount from about 2 to about 5%, vanadium in amount from about 2 to about 20%, molybdenum in amount from about 2 to about 15%, and manganese in amount from about 2 to about 8%, and balance titanium with incidental 10 impurities, which comprises heating said product for from about 15 minutes to about 2 hours at a temperature about that at which said alloy shows a minimum point on its yield strength, solution heat treating temperature curve, and rapidly quenching said product from said temperature thereby to provide as a characteristic thereof a yield strength to tensile strength ratio of between 0.25 to 0.75.

#### References Cited

##### UNITED STATES PATENTS

|           |         |               |       |          |
|-----------|---------|---------------|-------|----------|
| 2,554,031 | 5/1951  | Jaffee et al. | ----- | 75—175.5 |
| 2,575,962 | 11/1951 | Jaffee et al. | ----- | 75—175.5 |
| 2,596,485 | 5/1952  | Jaffee et al. | ----- | 75—175.5 |
| 2,675,309 | 4/1954  | Vordahl       | ----- | 75—175.5 |
| 2,726,954 | 12/1955 | Jaffee et al. | ----- | 75—175.5 |
| 2,777,768 | 1/1957  | Busch et al.  | ----- | 75—175.5 |
| 2,798,806 | 7/1957  | Jaffee et al. | ----- | 75—175.5 |
| 2,880,087 | 3/1959  | Jaffee et al. | ----- | 75—175.5 |
| 2,453,896 | 11/1948 | Dean          | ----- | 148—13   |
| 2,711,960 | 6/1955  | Methe         | ----- | 75—175.5 |
| 2,718,465 | 9/1955  | Herres        | ----- | 75—175.5 |
| 2,754,204 | 7/1956  | Jaffee et al. | ----- |          |
| 2,864,697 | 12/1958 | Busch et al.  | ----- |          |

##### FOREIGN PATENTS

|         |        |                |
|---------|--------|----------------|
| 718,822 | 3/1942 | Germany.       |
| 679,705 | 9/1952 | Great Britain. |

CHARLES N. LOVELL, Primary Examiner.